

## UNITED STATES PATENT OFFICE

JACK L. BITTER AND RICHARD ELSSNER, OF JOHNSON CITY, TENNESSEE, ASSIGNORS TO  
AMERICAN GLANZSTOFF CORPORATION, OF NEW YORK, N. Y., A CORPORATION OF  
DELAWARE

## YARN TREATMENT

No Drawing.

Application filed July 2, 1931. Serial No. 548,474.

Our present invention has to do with the production of the yarn of artificial filaments which possesses even shrinkage.

More particularly our new invention comprises the method whereby the yarn may be dried upon the usual hard spool and still not have the usual drawback of uneven shrinkage of the yarn body.

Other objects will become apparent from 10 a reading of the following specification.

Usually yarn from cellulosic solutions, after passing through the coagulating medium, is wound in the wet form upon a spool which might be any of the well known forms, 15 such as perforated, laminated, or corrugated. The threads of this yarn are then washed, and, for example in the viscose process, desulphurized, as well as bleached, etc. After the wet treatment, the yarn is usually dried by a 20 drier or a drying process which circulates hot air through and over the surfaces of the same while it is still on the spools. By following the usual processes the yarn is ordinarily allowed to dry both from the outer and 25 inner surface towards the middle thereof. By this process the outer and inner portion of the thread body are first dried and have a tendency to shrink and then the center portion is dried. Inasmuch as the innermost layers 30 rest upon a solid bobbin or spool, and the outermost layers are resting upon the middle layers, which are drying last, the outer and inner portions do not have sufficient chance 35 to shrink in the same way the middle layer does. This causes an uneven shrinkage or contraction of the filaments comprising the yarn body and is very undesirable.

Our present invention has to do with a new method of drying and treating the filaments 40 so that a high and uneven shrinkage or contraction is totally eliminated.

One method whereby our new process may be accomplished follows:

The yarn is extruded as usual and wound 45 upon any ordinary type of bobbin or spool. Then a cloth or other suitable air and liquid tight covering of sufficient thickness is wrapped about the spool so that all the moisture contained in the yarn must be dried out 50 from the inside. The spool is then placed in

the drier and allowed to dry as usual. This wrapping causes the inner and middle layers of the yarn to become dried first thereby giving the outer layers room within which to shrink. After thus drying the yarn body 55 upon the spool, the spool or bobbin is then placed upon a rewinding machine, as, for example, a twisting machine, a winding machine, etc., and the yarn wound upon another bobbin or spool, so that the resulting yarn 60 body is loose and room is allowed for shrinking. By this rewinding the position of the yarn body is changed about and the layers which were on the outside before are now upon the inner side. The spool is then rewet, 65 wrapped again with a sufficient amount of cloth or a water and air tight covering of suitable material so that moisture can only be taken out from the inside and again placed in the drier. This drying allows the inner 70 layers or the middle layers to dry first, as in the first case thereby giving the outer layer, which was before the inner layer, sufficient room within which to shrink to the same degree that was obtained in the other two layers. The performance of the second drying 75 gives a yarn body the parts of which are all evenly dried and therefore evenly shrunk.

Graphs have been made, depicting the evenness (or unevenness) of drying of artificial filaments when different processes are used. Results show that in the old direct spool process, described in paragraph four of the present specification, the drying produces a very 80 uneven shrinkage of the yarn or filaments being treated. A shrinking of approximately 3.4% on the inside of the spool, of approximately 2.5% on the outside, and varying percentages of shrinking, varying irregularly, 85 for the inner filaments, are indicated. However, when the outer surfaces of the spooled filaments are covered, usually with a flexible, water-tight covering, as indicated above, a more even shrinkage curve results. The 90 shrinkage when the applicants' present process is used more nearly approaches that of skein drying. Because drying the filaments in skein form involves many extra steps and is comparatively expensive, it may be easily 95 100

seen that the present process covers a great step forward in the art.

Although we have hereinbefore described specifically one method whereby the yarn <sup>5</sup> might be dried in one direction only, rewet, rewound, and dried in the other direction because of the changed space of the yarn, it must be understood that we do not desire to limit ourselves to this specific modification <sup>10</sup> but the invention includes within its purview whatever changes that come within the terms or spirit of the appended claims.

Having now fully set forth our invention <sup>15</sup> as required by the patent statutes, what we desire to claim is:

1. In a method for drying artificial filaments wound upon a perforated bobbin, the step of removing the moisture from the yarn body in one direction only by first covering <sup>20</sup> the outer surface of the filaments with an impermeable covering, and then applying a drying medium to the inner side only of the bobbin so that the yarn body dries from the inner side only.

<sup>25</sup> 2. In a process for drying artificial yarn which has been collected on a foraminous holder, the step of covering the outer surface of the yarn body with an impermeable covering, and applying the drying medium to the inner side of the holder so that the yarn body dries only from the inner side.

<sup>30</sup> 3. A process as set forth in claim 1, wherein the yarn is rewound onto another bobbin, rewet, and then redried from the inside only.

<sup>35</sup> 4. The process as set forth in claim 2, wherein the yarn is then rewound upon another similar holder, so that a loose winding results, and the filaments are then rewet and redried.

<sup>40</sup> 5. In a process of the class described, the steps of wrapping wet artificial yarn wound upon a perforated spool with an impermeable covering, and then applying a drying medium to the inner surface of the spool, thus <sup>45</sup> drying the yarn from the inner side of the spool only.

<sup>50</sup> 6. In a process for drying artificial yarn, filaments, etc., upon a foraminated spool, the steps of covering the outer surface of the filaments etc., with an impermeable covering, drying the same from the inside only by introducing a drying medium to the inner side of the spool, rewinding onto another spool or bobbin, rewetting the filaments, and then redrying, with the use of an impermeable cover, from the inside of the spool only.

In testimony whereof we affix our signatures.

DR. JACK L. BITTER.  
DR. RICHARD ELSSNER.